

Dec. 24, 1935.

H. HANUSCH

2,025,050

CEMENTING AGENT FOR STEEL AND IRON

Filed Nov. 3, 1931



Inventor:  
Hugo Hanusch  
by his Attorney  
Hauson & Hauson

## UNITED STATES PATENT OFFICE

2,025,050

## CEMENTING AGENT FOR STEEL AND IRON

Hugo Hanusch, Berlin, Germany, assignor to E. F.  
Houghton & Company, Philadelphia, Pa.Application November 3, 1931, Serial No. 572,859  
In Germany November 8, 1930

10 Claims. (Cl. 148—27)

This invention relates to a cementing composition for steel and iron and more particularly it relates to carbonaceous cementing baths which are relatively poor in cyanides or even free there-  
5 of.

For the hardening and cementing of steel and iron there are used generally solid carburizing agents as well as liquid salt baths. The advantages and disadvantages of both compositions are  
10 sufficiently known.

The salt baths used for the cementing or hardening process at the present time are characterized by a high content of cyanide compounds. In order to increase the penetrating effect of the  
15 cementing bath it had heretofore been necessary to increase the content of cyanide in the bath. In consequence of this, for instance, cementing salts having a content of sodium cyanide of 45, 75 and even up to 98% are being put on the market  
20 by prominent concerns.

However, on account of its poisonous qualities a salt bath of this kind is a continuous source of danger.

In a general way my invention is based upon  
25 the discovery that it is possible to make cementing salt baths and solid cementing agents (carburizers) which contain either no cyanogen at all or little cyanogen and in spite of this possess a great cementing penetration, if as a carbonaceous  
30 agent a carbon is used to which there have been imparted by previous physical or chemical treatment, special properties expediting the process of cementation.

Up to the present time it had not been possible  
35 to incorporate in the bath a quantity of carbon sufficient to obtain a deep cementation. It has been found that the kind of carbon which has so far been used in cementing baths would separate from the salts and rise to the surface of the bath,  
40 where it will burn quickly through the action of the oxygen of the air. In consequence of this no intensive carburization of the work-piece could be attained.

My invention is based upon the discovery that  
45 a deep cementing effect can be attained by means of carbon which is especially suitable for this purpose, that is a carbon which has been subjected to a physical or chemical treatment with a view to activating said carbon, thereby reducing  
50 its combustibility either in the manner described in the German Patents 453,972 of December 28, 1927, 466,358 of October 5, 1928, and 488,669 of January 3, 1930 or in some other way.

Such carbons are termed herein and in the  
55 claims "activated carbon of low combustibility".

These carbons, upon being subjected to the full flame of a Bunsen burner for a period of two hours, leave a residue of non-combustibles of at least 50% by weight of the original sample as distinguished from the ordinary activated carbon, which, upon subjection to the same tests, leaves a considerably smaller percentage of non-combustibles.

In accordance with the disclosure of German Patent No. 453,972, ordinary carbon from any source is heated to glowing in a suitable vessel with porous or gas-permeable walls, and thereafter submitted while glowing to the action of oxygen or oxygen-containing gases passed through the carbon mass or through the walls of 10 said vessel. The German Patent No. 466,358 describes an improvement of the process of German Patent No. 453,972 by which even less combustible activated carbon is prepared by treating granular carbon from any source with a water-glass solution followed by precipitation of the silicic acid by the action of acids prior to the treatment of the carbon as described in the main German Patent No. 453,972. An activated carbon product having a silicic acid skeleton is produced which possesses great mechanical strength and may be used advantageously in chemical reactions without losing its shape. The German Patent No. 488,669 describes another method for manufacturing a highly activated carbon of low 20 combustibility. The carbon is treated with inorganic substances in solution, or as colloids, which substances exert a combustion-decreasing influence, and are precipitated as insoluble oxides by a carbonization process. Prior to carbonization, other substances are also added, such as zinc chloride or phosphoric acid to increase the activity of the carbon. It will be noted that all of these processes produce an activated carbon of 30 low combustibility which has proved, in accordance with the present invention, to give novel and unexpected results when employed in cementing salt baths.

When using carbon of this kind it will be possible to incorporate a quantity of carbon amounting to as much as 10% in the cementing bath and thereby to obtain an exceptional penetration. It will also be possible when using such cementing baths to work at temperatures above 900° C. which will greatly expedite the cementing process 40 but could not be used easily in the present cementing baths, as the latter are liable to undergo decomposition at these temperatures.

I have succeeded in making up salt baths in the aforementioned manner which contain only from 50

4 to 6% of pure cyanogen and in spite of this will effect a cementation which heretofore could hardly be attained with salts containing from 75 to 98% of sodium cyanide. The poisonous and dangerous character of these salt baths will thus be quite considerably reduced with the result that these new baths do not involve more danger than many machines and processes used in the modern industry. In addition to this, such baths are 10 materially cheaper than salt baths having a high content of cyanide.

The baths may be made up in the usual manner and, besides chlorides, also carbonates and alkalies may be used. The cyanide compounds 15 contained in the baths may consist of sodium cyanide or potassium cyanide, potassium ferrocyanide, calcium cyanamide and so forth.

The following two examples are given to show how the new salt baths may be composed.

|                                        | Per cent |
|----------------------------------------|----------|
| Sodium cyanide                         | 8        |
| Sodium chloride                        | 65       |
| Potassium chloride                     | 19       |
| Activated carbon of low combustibility | 8        |

*Example 1*

|                                        | Per cent |
|----------------------------------------|----------|
| Sodium cyanide                         | 8        |
| Sodium chloride                        | 62       |
| Potassium chloride                     | 18       |
| Activated carbon of low combustibility | 8        |
| Carbonate of barium                    | 2        |
| Caustic soda                           | 2        |

35 On the basis of experiments I have ascertained that with properly composed baths there will be an excellent cementation, also in case of solid cementing agents, if at the same time activated carbon of low combustibility is used in 40 considerable quantities.

*Example 3*

|                                        | Per cent |
|----------------------------------------|----------|
| Ordinary carbon                        | 85       |
| Potassium ferro-cyanide                | 5        |
| Activated carbon of low combustibility | 5        |
| Carbonate of barium                    | 5        |

*Example 4*

|                                        | Per cent |
|----------------------------------------|----------|
| Ordinary carbon                        | 90       |
| Activated carbon of low combustibility | 5        |
| Carbonate of barium                    | 5        |

55 I have further found that the time required for the cementing process may be considerably reduced, if the cementing bath is closed hermetically and kept under pressure.

In the drawing I have shown in diagrammatic vertical section an apparatus which is suitable 60 for carrying out my novel process for cementing steel and iron under pressure.

The container 1 may be hermetically closed by means of a cover 2 and packings 3, as indicated in the drawing. The gases which are being developed at the cementing temperatures will cause an over-pressure to arise within the container 1 which over-pressure may be regulated by means of the valve 4, 5 and controlled by a pressure gauge 6. The work-piece 7 to be subjected to the 65 cementing process is suspended within the container 1 and kept immersed in the bath 8 within the container 1. As cementing baths with which the process of cementing may be carried out under pressure there may be used baths of the aforementioned kind, as well as all other cementing

baths which had heretofore been used, especially also cyanogen containing cementing agents known in commerce under various trade-marks or the various cyanide hardening compounds sold under the name of their manufacturers.

I claim:

1. An iron and steel cementing bath composition, molten at cementing temperatures and containing material capable of supplying carbon to the metal at said temperatures, comprising an alkali metal cyanide in the neighborhood of 8%, sodium chloride in the neighborhood of 62% to 65%, potassium chloride in the neighborhood of 18% to 19%, and an activated carbon of low combustibility in the neighborhood of 8%.

15 2. An iron and steel cementing bath composition, molten at cementing temperatures, and containing material capable of supplying carbon to the metal at said temperatures, comprising a salt inert to the iron and steel molten at cementing 20 temperatures as the major ingredient of said composition, and at least 4% of activated carbon of low combustibility, the last named ingredient supplying carbon to the metal at cementing temperatures.

25 3. An iron and steel cementing bath composition, molten at cementing temperatures and containing material capable of supplying carbon to the metal at said temperatures, comprising a salt inert to the iron and steel molten at cementing 30 temperatures as the major ingredient of said composition, a cyanide compound and at least 4% of activated carbon of low combustibility, the last named ingredients supplying carbon to the metal at cementing temperatures.

35 4. An iron and steel cementing bath composition, molten at cementing temperatures and containing material capable of supply carbon to the metal at said temperatures, comprising a mixture of salts inert to the iron and steel molten at 40 cementing temperatures as the major ingredient of said composition, alkali metal cyanide and at least 4% of activated carbon of low combustibility, the last named ingredients supplying carbon to the metal at cementing temperatures.

45 5. An iron and steel cementing bath composition, molten at cementing temperatures and containing material capable of supplying carbon to the metal at said temperatures, comprising a salt inert to the iron and steel molten at cementing 50 temperatures as the major ingredient of said composition, alkali metal cyanide in the neighborhood of 8% and at least 4% of activated carbon of low combustibility, the last named ingredients supplying carbon to the metal at cementing temperatures.

55 6. An iron and steel cementing bath composition, molten at cementing temperatures and containing material capable of supplying carbon to the metal at said temperatures, comprising a salt inert to the iron and steel molten at cementing 60 temperatures as the major ingredient of said composition, alkali metal cyanide in the neighborhood of 8% and activated carbon of low combustibility between 4% and 10%, the last named ingredients supplying carbon to the metal at cementing temperatures.

65 7. An iron and steel cementing bath composition, molten at cementing temperatures and containing material capable of supplying carbon to the metal at said temperatures, comprising a salt inert to the iron and steel molten at cementing 70 temperatures as the major ingredient of said composition, alkali metal cyanide in the neighborhood of 8% and activated carbon of low combustibility in the neighborhood of 8% and activated carbon of low com-

5

15

25

35

45

50

55

65

75

bustibility in the neighborhood of 8%, the last named ingredients supplying carbon to the metal at cementing temperatures.

- 5 8. An iron and steel cementing bath composition, molten at cementing temperatures and containing material capable of supplying carbon to the metal at said temperatures, comprising an alkali metal cyanide in the neighborhood of 8%, sodium chloride in the neighborhood of 62%, potassium chloride in the neighborhood of 18%, activated carbon of low combustibility in the neighborhood of 8%, barium carbonate in the neighborhood of 2%, and caustic soda in the neighborhood of 2%.
- 10 9. An iron and steel cementing bath composition, molten at cementing temperatures, and containing material capable of supplying carbon to the metal at said temperatures, comprising a salt inert to the iron and steel molten at cementing
- 15

temperatures as the major ingredient of said composition, and at least four percent of activated carbon of low combustibility containing inorganic material within its pores, the said activated carbon supplying carbon to the metal at 5 cementing temperatures.

- 10 10. An iron and steel cementing bath composition, molten at cementing temperatures, and containing material capable of supplying carbon to the metal at said temperatures, comprising a salt 10 inert to the iron and steel molten at cementing temperatures as the major ingredient of said composition, and at least four percent of activated carbon of low combustibility having a silicic acid skeleton, the said activated carbon supply- 15 ing carbon to the metal at cementing tempera- tures.

HUGO HANUSCH.